

## UNITED STATES PATENT OFFICE

THOMAS R. HEYWARD, JR., OF PITTSBURGH, PENNSYLVANIA

## APPARATUS FOR HEAT-TREATING METAL ARTICLES

No Drawing.

Application filed July 19, 1929. Serial No. 379,584.

This invention relates to the art of heat treating metals. It is concerned not only with new and improved apparatus for heat treating metals, particularly steel in the form of elongated relatively thin articles such as sheets or strips, but it is also concerned with a new and improved step or steps in the heat treatment of metals and in the operation of furnaces for heat treating metals in the above described form.

Heretofore thin elongated metal articles, particularly steel sheets and strips, have been heat treated by being passed on waster sheets, composed of iron or steel and, for example, of 18 gauge thickness, through heat treating furnaces provided with suitable conveying means which engaged and carried the waster sheets.

The waster sheets have been employed to space the articles being treated from the conveying mechanism in the furnace primarily for the purpose of preventing pittings or surface defects on the articles which often results from the presence of lumps in the form of complex oxides of considerable hardness adhering to the conveying mechanism. These waster sheets, which are usually composed of steel, oxidize and scale very rapidly, due to the high heat maintained in the furnace so that after a very few passes through the furnace the surfaces of the waster sheets become more or less completely covered with scale which flakes off as the steel wasters are repeatedly used. Such scale particularly on the lower surface of the sheet is dislodged from time to time by striking the conveyor mechanism and falls below the conveyor mechanism where it accumulates on the hearth of the furnace. This results in that the amount of heat reflected from the hearth is decreased and in time the hearth is so filled with scale that the furnace must be shut down, cooled off and the scale removed, a procedure that requires several days' time.

The scale on the upper surface of the steel waster sheet, which comes in contact with the metal articles being heat treated, is harder at the highest temperatures than the sheets being treated and tends to scratch

or form pits in the metal articles. The scaled waster sheets also are relatively poor conductors of heat as compared with the unscaled waster sheet. Consequently the heat from the waster sheet is not transmitted uniformly throughout the entire surface of the waster sheet to the articles carried thereon with the result that the articles which rest on such scaled waster sheets are non-uniformly heated and consequently the physical properties of the resultant articles are not uniform throughout. This non-uniformity of heating destroys the prime reason of such a furnace as it is highly desirable that the articles should be uniformly heat-treated throughout and that the physical properties should be substantially the same throughout the articles.

Moreover, the iron or steel waster sheets used heretofore have an exceptionally short life, due to the scaling tendency, and such waster sheets which have been passed through a continuous normalizing furnace for perhaps less than two hundred times are entirely useless for further use. In addition to this rapid deterioration of the iron or steel waster sheets, these sheets are difficult to handle after they have passed through a furnace a small number of times because of the formation of loose and splintery scale on the edges, together with the surface scale thereof which readily cut the hands of workmen who handle the waste sheets at the exit and entering ends of the furnace and likewise due to their roughness of scale and splinters often scratch the articles as they are removed from the waster at the exit end of the furnace.

The usual prior practice with steel waster sheets has been to use sheets of about 18 gage, (.050") to 20 gage (.037"). They can be used longer than thinner sheets before the scaling has reduced them to such a thinness that the incrustations on the conveyor will penetrate through them and pit or mar the article thereon. An important disadvantage, however, is that the steel waster sheets will thus vary in thinness and amount of scale. For example, after some use certain sheets will be discarded as no longer

useful and replaced by new sheets. Then the old sheets may be reduced to 20 gage (.037") or less while the new sheets are thicker and carry less scale. As time goes on the sheets for a given furnace may be all of different thicknesses and of different degrees of scaling. The result is that the articles being treated are not uniformly heated and the product will vary in physical properties.

By my invention I start with thinner carrier sheets, for example 24 gage (.025") which, due to their properties, resist penetration by the incrustations as well or better than the thicker steel waster sheets, and repeatedly use my carrier sheets many times as long as the steel waster sheets can be used so that replacements are decreased and the resultant product is of a much more uniform character.

Furthermore, a scaled steel waster sheet does not dissipate heat as rapidly as my non-scaling carrier sheet. This has a marked effect on grain growth in the article being heat treated, particularly in normalized sheets or strip metal, and results in larger grains in the parts of articles contacting with the scaled steel waster than in the upper or more quickly cooled metal, the variance in grain growth depending on the thickness and amount of scale present on the steel waster sheet. With my alloy carrier sheets the heat is dissipated rapidly therefrom and undesired grain growth is prevented in the metal of the articles contacting therewith.

Wide differences in results between the steel waster sheets and my alloy carrier sheets is even more pronounced than above noted when two or more metal article sheets are carried through the furnace in stacked relation in that the heat dissipation from the bottom article sheet is retarded by the article sheets thereabove and must, therefore be increased through the alloy carrier or steel waster sheets in order to obtain the same physical and microstructural properties in the bottom sheet as are obtained in the article sheets thereabove. My alloy carrier sheets are much better adapted to such heat dissipation than the steel waster sheets whether or not the latter are scaled.

By means of the present invention I am able to overcome the disadvantages present in the waster sheets of the prior art, to obtain a carrier sheet which will be much thinner than the steel waster sheets, and have many times the length of life of the prior art waster sheets, and which will not only be easier to handle, due to the lighter weight and absence of slivers and scale, but which will also be capable of transmitting heat more quickly than the steel waster sheets and also substantially uniformly throughout its entire surface to the articles in contact

therewith for substantially the full life of the carrier sheets.

My improved non-scaling carrier sheet possesses another distinct advantage when used with certain compositions of conveyors in a furnace burning fuel which contains considerable amounts of sulphur. Certain conveyor compositions are attackable by the joint action of sulphur and scale, for example chrome nickel compositions high in nickel. If such conveyor compositions are used with steel carrier sheets which scale badly and with sulphur containing fuel the conveyors rapidly deteriorate. With my present non-scaling carrier sheets, however, the scale is practically eliminated and the life of the carriers correspondingly prolonged, as the action of the sulphur gas alone is less detrimental than sulphur gas in the presence of iron oxide.

In practicing my invention I form a relatively thin carrier sheet of, for example, 24 gage metal and of the desired size and configuration of a metal or metal composition, which is highly resistant to oxidation at high temperatures as compared with iron or steel. Such a composition which has been found in use to be satisfactory for long continued use, consists predominantly of iron and contains from fifteen percent to about thirty percent of chromium. Other suitable compositions consist of iron with about fifteen percent to thirty percent of chromium and from about five to about fifteen percent of nickel. Part of the chromium may be replaced by nickel. One preferred composition consists of iron with about twenty-eight per cent of chromium due to its greater resistance to oxidation at high operating temperatures and also to greater resistance to the varying fuel compositions. Another satisfactory composition contains about eighteen percent chromium and eight percent nickel.

My improved carrier sheets are employed in the method of operating a metal heat treating furnace or in the method of continuously heat treating articles as for illustrative purposes, a continuous normalizing furnace with a process as follows.

When a normalizing furnace of the continuous type that is a type in which the articles move from the entrance to the exit of the furnace is being used for continuously normalizing sheet metal, alloy carrier sheets of my invention are placed on the conveyor mechanism of the furnace at the charging end and the sheet articles to be treated are placed thereon. The carrier sheets thus space the articles from the conveyor mechanism which would mar the surface of the article due to the presence of oxide lumps previously described. The conveyor mechanism then moves the carrier sheets and articles thereon through the fur-

- nace, and both the articles and carrier sheets are heated to the desired temperature and then cooled. When the carrier sheets and articles emerge from the exit end of the furnace the articles are removed from the carrier sheets, which are then ready for further treatment or use. The carrier sheets are then returned to the charging end of the furnace for a repeat of this process.
- 5 During the passage of the carrier sheets and articles thereon through the furnace, the carrier sheets are heated to approximately the temperature of the articles thereon and the heat thus absorbed by the carrier sheets is transmitted substantially uniformly from the entire upper surface of the carrier sheets to all surfaces of the articles contacting therewith. This results in the latter being uniformly heated by the carrier sheets and 10 in the articles being substantially and uniformly heated treated throughout. As the articles cool in the cooling zone of the furnace they transmit heat to the carrier sheets for substantially the entire upper surface of 15 the latter and such heat is dissipated by the carrier sheets more or less uniformly from its lower surface so that substantially the entire surface of the articles in contact with the carrier sheets is uniformly cooled and 20 certain parts are not cooled more slowly nor more rapidly than other parts as often occurs with badly scaled steel waster sheets.
- 25 Moreover the chrome-iron carrier sheet absorbs and dissipates its heat more rapidly due to its thinness, and its freedom from scale than a steel waster which is a marked advantage. My thinner non-scaling alloy carrier sheet also shapes itself to the articles thereon and brings more of its non-scaled 30 surface into contact with the articles more quickly than does the thicker and scaled steel waster sheets and consequently heats the articles thereon more completely, quickly and uniformly than does the steel sheets.
- 35 Having thus described my invention so that those skilled in the art may be enabled to practice the same, what I desire to secure by Letters Patent is defined in what is claimed. It being understood that various 40 changes in the foregoing detailed description may be made by those skilled in the art without departing from the spirit and scope of my invention.
- 45 What is claimed is—
- 50 1. A carrier sheet for use in a heat treating furnace comprising iron containing between about fifteen percent and about thirty percent of chromium, the sheet being substantially non-scaling at furnace operating 55 temperatures as compared with steel waster sheets and possessing throughout substantially its full serviceable life the property of transmitting heat substantially uniformly to and from all surfaces of the article sheet 60 65 making contact therewith.
2. In combination with a continuous heat treating furnace and conveyor means in the furnace for moving through the furnace metal to be heat treated, a carrier sheet engageable with and carried by the conveyor means and adapted to carry thereon and 70 through the furnace metal articles to be treated, the carrier sheet being composed of an alloy having high resistance to oxidation and scaling as compared to iron or steel at the temperatures to which it is subjected in the furnace, and having throughout substantially its full serviceable life the property of transmitting heat to articles thereon substantially uniformly to and from all surfaces of the articles being treated which 75 make contact with the alloy carrier sheet.
- 75 In testimony whereof I hereunto affix my signature this 13th day of July, 1929.
- 80 THOMAS R. HEYWARD, JR.
- 85
- 90
- 95
- 100
- 105
- 110
- 115
- 120
- 125
- 130